

March 27, 1934.

O. C. RALSTON

1,952,727

FROTH FLOTATION

Filed Oct. 26, 1929

Fig. 1



Fig. 2



INVENTOR

Oliver C. Ralston  
BY

Tennie, Davis, Marvin & Edmonds  
HIS ATTORNEYS

## UNITED STATES PATENT OFFICE

1,952,727

## FROTH FLOTATION

Oliver C. Ralston, Clarkdale, Ariz., assignor to  
 United Verde Copper Company, Clarkdale,  
 Ariz., a corporation of Delaware

Application October 26, 1929, Serial No. 402,635

8 Claims. (Cl. 209—164)

This invention relates to the control of froth in flotation and has for an object the provision of an improved method and apparatus for controlling froth formation and froth discharge and inhibiting the flotation of gangue and other undesirable minerals.

According to the heretofore customary practices, the ore or mixture of minerals in the form of a pulp is subjected to agitation in the presence of frothing and mineral collecting agents in cells provided with overflow lips and having froth forming compartments adjacent the overflow lips. The froth produced contains the valuable minerals or a portion thereof and it is permitted to overflow into suitably disposed launders which are provided for the purpose of conducting the froth to suitable settling and thickening apparatus.

The ore being treated usually contains more than one mineral capable of being floated by means of the reagents employed. In some cases, the ore contains two or more valuable minerals to be recovered and, usually, a readily floatable mineral such as pyrite which it is desirable to reject. Flotation operations are therefore so conducted as to promote the flotation of one or more minerals while inhibiting the flotation of other minerals. This is accomplished through control of the reagents employed, that is, by employing reagents having differing degrees of affinity for the various minerals in the proper proportions and amounts. In some cases, the flotation operations are conducted in stages in different ones of which the concentrate obtained is composed largely of different minerals.

The heretofore customary type of selective or differential flotation operation, therefore, required a very careful control of the type and amount of reagent used for the complete operation or for any stage of the operation in the event that different minerals were recovered in different stages. The usual reagents employed are capable of effecting flotation of any of the minerals contained in the ore, but since the affinity of a particular reagent may be greater for one mineral than for another it is at least theoretically possible to selectively float one mineral from a mixture through properly controlling the amount of reagent employed and/or the conditions under which the reagent is employed.

In spite of the different affinities of various reagents for different minerals, it is virtually impossible in commercial operations to effect a complete separation of the different minerals in the primary cells even when the utmost care is

exercised in adding the proper types and amounts of reagents. The primary froth usually contains some of all of the minerals present in the pulp feed. This is due to the continuously varying quality of the feed, the practical impossibility of adding only the exact amount of reagent required and the practical impossibility of continuing the operations for a sufficient length of time to permit definite selective action. Some undesirable minerals and gangue are also present in the water from the pulp which is present in the bubble films.

Voluminous froths are produced at times during the course of normal flotation operations. Thus, a flotation operation may proceed satisfactorily for a relatively long period with the production of a froth of a type which is satisfactory with respect to volume and mineral content and then suddenly or gradually, by some agency not under the direct control of the operator, be converted to an unsatisfactory operation producing a voluminous froth carrying excessive amounts of undesirable minerals and gangue. Such changes are usually caused by changes in the character of the ore, and correction can generally be made by adjustment of the amount or type of reagent being added. However, it is rather difficult to adjust the rate of addition and character of reagents to compensate for all changes in the character of the ore which affect the volume and mineral content of the froth.

In the operation of the usual flotation cell, a layer of froth several inches in thickness is present in the froth forming compartment. The bubbles forming the upper or surface portion of the froth layer and, particularly, those adjacent the source of agitation which produces the frothing effect, are generally larger than the remaining bubbles. The large bubbles and other fast forming bubbles adjacent the source of agitation appear to contain the larger proportion of gangue and undesirable minerals, but all bubbles contained in the froth are contaminated to some extent with undesirable minerals and gangue.

According to the method of the present invention, the froth is subjected to a type of treatment in the froth forming compartment as a result of which the mineral burdens of the froth overflowing may be controlled and regulated.

The apparatus of the invention comprises a flotation cell having in combination therewith means for treating the bubbles so as to control the nature of the solid materials in the bubble films of the froth overflowing the cell.

The present invention provides for the elimi-

60

65

70

75

80

85

90

95

100

105

110

nation of undesirable matter from the froth by substituting a liquid of the desired composition for the contaminated liquid of the bubble films as formed; by destroying surface bubbles and 5 transferring their mineral burdens to other bubbles; or by combined substitution of film substance and destruction of surface bubbles. The invention also contemplates the treatment of the bubbles of the froth with relatively small particles of mineral of the type for which the reagent or combination of reagents being used has the greater affinity, to effect a substitution of such mineral particles for the undesirable minerals in the froth. According to the process of the invention, the surface bubbles of froth on bodies of pulp in froth forming compartments are subjected to the action of agents capable of effecting the desired changes in the compositions of the bubble films or the mineral burdens of the bubbles in the froth. Such agents may be applied, conveniently, in the form of sprays. The spray may comprise, for example, water, a mixture of air and water, a solution of a reagent capable of influencing the rejection of undesirable minerals, 10 or particles of finely divided solid material alone or mixed with any suitable fluid.

The force of the spray to be directed against the surface bubbles will be determined by the effect desired. For example, if only a substitution 15 of film substance is desired, a gentle or low velocity spray which will cause a minimum breaking of bubbles should be employed. If the surface bubbles are to be broken for the purpose of showing their mineral burdens upon the lower bubbles a high velocity spray should be employed. A high velocity spray may be produced conveniently by means of a liquid atomizer consisting of an air nozzle connected to a source of supply of air under pressure, and a liquid supply nozzle having 20 its discharge opening disposed immediately adjacent the discharge opening of the air nozzle. A combined film substance substituting and bubble breaking effect will be achieved when a high velocity spray containing a liquid is employed. 25 This effect may be varied by varying the velocity of the spray and/or the volume of liquid contained therein.

The invention will be better understood from a consideration of the following description in conjunction with the accompanying drawing, in which

Fig. 1 is a sectional elevation of a flotation cell having spray devices disposed above the froth forming compartment; and

Fig. 2 is a side elevation of the apparatus shown in Fig. 1.

The flotation cell 10 is of the pneumatic type in which agitation of the pulp containing the desired reagents is effected by means of downwardly directed air streams entering the pulp body through centrally disposed conduits 11. The flotation cell is provided with froth forming compartments 12 having overflow lips 13. Concentrate launders 14 are disposed adjacent the overflow lips 13 and are adapted to receive the froth passing over the lips 13.

A number of spray devices or atomizers 17, each comprising a conduit 15 for supplying gas under pressure, and a conduit 16 for supplying a liquid are disposed above each of the froth forming compartments and connected to suitable sources of supply of gas under pressure and liquid (not shown). The atomizers may be adjustably mounted in order that the particles of fluid 70 issuing therefrom may be directed against the

surface of the froth at any desired point and/or at any desired angle. Suitable valves may be provided in the gas and liquid conduits for controlling the flow of gas and liquid.

Spray pipes 20 may be provided instead of or in addition to the atomizers 17. The spray pipes 20 extend transversely of the flotation cell and are connected to liquid supply headers 21 extending longitudinally of the flotation cell. The spray pipes 20 are perforated in such a manner that fine streams or small droplets of liquid may be directed against the surface of the froth at points removed from the overflow lip. The rate of flow of liquid from the apertures in the pipes 20 may be controlled by means of the valves 22 in the lines 23 which are connected to a source of supply (not shown).

In the operation of the apparatus of the invention, the froth formed rises to the surface of the pulp body in the froth forming compartments and passes over the overflow lips into the concentrate launders.

When a gentle spray of pure water is applied, for instance by means of spray pipes 20, the water tends to pass downwardly through the 100 layer of froth and in so doing it becomes substituted in the films of the bubbles with which it comes into contact for the liquid of which the films were originally formed. The displaced liquid together with the undesirable gangue and 105 other materials contained therein passes downwardly into the pulp body.

When a high velocity spray capable of rupturing the surface bubbles is employed, the mineral burdens of the ruptured bubbles are shown 110 downwardly upon the bubbles beneath the surface. When the released minerals come into contact with the lower bubbles, the particles of the mineral for which the reagent employed has the greater affinity will displace particles of the 115 mineral or minerals for which the reagent has the lesser affinity with the result that the desired mineral will be concentrated upon the lower bubbles which pass outwardly beyond the range of the fluid streams.

The effect of the application of finely divided minerals to the froth is similar to the effect achieved by using a high velocity spray, that is, a displacement and rejection of undesirable minerals is achieved. The mineral particles may be 125 applied in any desirable manner. A pulp of a high grade concentrate obtained in the particular operation involved may be used conveniently.

Solutions of reagents may be applied in any desired manner. Thus, lime solution may be 130 sprayed gently over the surface of the froth to produce the combined effect of displacing the original film substance and causing an additional rejection of pyrite, or the reagent may be applied in the form of a high velocity spray.

It may be desirable to provide merely for breaking some of the bubbles of the froth without incorporating any extraneous material. In such cases a mechanical device capable of rupturing the bubbles, or a spray comprising an inert gas, 140 or finely divided solid may be employed.

The method of the present invention provides a desirable supplement to reagent control, and it may be utilized continuously or intermittently as conditions warrant. The process may be 145 utilized continuously to supplement reagent control, permitting control of the amount and character of the froth without necessitating close control of reagents.

It permits the use of a constant amount of 150

- reagent and provides control of frothing conditions which arise as a result of changes in the character of the ore or the presence of unknown components in the reagents. Since the process 5 of the invention provides froth control, it may be utilized in conjunction with inferior reagents, and it permits the use of reagents which produce tough froth.
- The method of the invention may be used to 10 particular advantage in flotation operations conducted in pneumatic cells. The froth produced in such cells is a primary froth containing relatively large amounts of undesirable minerals, as distinguished from residual froth of cells employing mechanical agitation which has been subjected to the beating action of impeller blades. The process may be utilized for controlling frothing conditions in either rougher or cleaner cells or both, but its use in conjunction 15 with cleaning operations will generally be sufficient. When the process is used in conjunction with cleaning operations, close control of frothing conditions in the rougher operations is unnecessary.
- 20 I claim:
1. In a froth flotation process, the method of controlling the character of the froth which comprises directing a spray containing particles of solid matter against a portion of the froth in the 25 froth forming compartment of a flotation cell to effect a rejection of undesirable material contained therein.
2. In a froth flotation process, the method of controlling the character of the froth which comprises directing a spray containing particles of solid matter against the froth in the froth forming compartment of a flotation cell to break a 30 portion of the bubbles forming the froth and shower their mineral burdens on other bubbles.
3. In a froth flotation process, the method of controlling the character of the froth which comprises spraying the upper surface of a layer of froth on the surface of a body of pulp in a 35 flotation cell with a liquid capable of entering the froth as a substitute for the bubble films, and regulating the spraying operation to effect a substitution of the liquid of the spray for the bubble 40 films.
4. In a froth flotation process, the method of controlling the character of the froth which comprises directing a liquid spray against a layer of froth in the froth forming compartment of a flotation cell to break bubbles comprising the 45 upper portion only of the froth layer and shower their mineral burdens on bubbles comprising the lower portion of the froth layer, thereby to produce a froth of improved quality through replacement of undesired minerals in the lower bubbles with desired minerals released through breakage of the upper bubbles.
5. In a froth flotation process, the method of controlling the character of the froth which comprises directing a high velocity spray comprising minute particles of liquid against a layer of froth in the froth forming compartment of a flotation cell to break bubbles comprising the upper portion only of the froth layer and shower their mineral burdens on bubbles comprising the lower portion of the froth layer, thereby to produce a froth of improved quality through replacement of undesired minerals in the lower bubbles with desired minerals released through breakage of the upper bubbles.
6. In a flotation operation in which a mineral bearing froth is produced in a flotation cell and passes from the zone of production through a relatively quiescent zone on the surface of a pulp body to a point at which it is removed from the cell, the improvement which comprises spraying the froth while passing through the relatively quiescent zone with a liquid capable of entering the froth as a substitute for the bubble films, and regulating the spraying operation to effect a substitution of the liquid of the spray for the bubble 50 films.
7. In a flotation operation in which a mineral bearing froth is produced in a flotation cell and passes from the zone of production through a relatively quiescent zone on the surface of a pulp body to a point at which it is removed from the cell, the improvement which comprises applying to the froth while passing through the relatively quiescent zone an agent capable of entering the bubble structure to effect a rejection of undesirable matter contained therein, and regulating the operation to effect the rejection of undesirable matter from the froth.
8. In a froth flotation process, the step which comprises mechanically breaking the uppermost bubbles of a layer of froth on a body of pulp in a flotation cell without breaking the lowermost bubbles to shower the mineral burdens of the uppermost bubbles upon the lowermost bubbles and thus cause a displacement of undesired minerals contained in the lowermost bubbles by means of minerals released from the uppermost bubbles through breaking.
- OLIVER C. RALSTON.
- 55
- 60
- 65
- 70
- 75
- 80
- 85
- 90
- 95
- 100
- 105
- 110
- 115
- 120
- 125
- 130
- 135
- 140
- 145
- 150